

# UNITED STATES PATENT OFFICE.

PLUMER WHEELER, OF CHESTER, PENNSYLVANIA, ASSIGNOR TO THE E. I. DU PONT DE NEMOURS POWDER COMPANY, OF WILMINGTON, DELAWARE, A CORPORATION OF NEW JERSEY.

## METHOD OF PRODUCING HIGH-EXPLOSIVE COMPOUNDS.

No. 901,504.

Specification of Letters Patent.

Patented Oct. 20, 1908.

Application filed August 10, 1906. Serial No. 329,958.

*To all whom it may concern:*

Be it known that I, PLUMER WHEELER, a citizen of the United States, residing at Chester, county of Delaware, and State of 5 Pennsylvania, have invented a new and useful Improvement in Methods of Producing High-Explosive Compounds, of which the following is a full, clear, and exact description.

10 In recent years there have been proposed quite a large number of explosive compositions consisting largely of ammonium nitrate with combustible matters of different kinds, such as, resinous compounds, oils, organic 15 nitro-compounds, or mixtures of these compounds, etc. An example of such composition is a mixture of ammonium nitrate, dinitronaphthalene and trinitrotoluene. One great draw-back in the use of these explosives has been the fact that they are apt to be 20 of uncertain sensitiveness, sometimes failing to explode with even a very strong detonator. I have discovered the reason for lack of sensitiveness of these explosives. The 25 method, as ordinarily carried on, to produce these explosive compositions is to mix the ammonium nitrate with the combustible matters at a temperature only sufficient to liquefy such resinous compounds, oils, or organic 30 nitro compounds. I have discovered that if a temperature of mixing be used in excess of that necessary to liquefy these combustible matters, but not high enough to liquefy the ammonium nitrate, the sensitiveness of the 35 explosives progressively increases the higher the temperature and the best results are obtained as the temperature approaches the melting point of the ammonium nitrate.

I have obtained substantially good results 40 at as low a temperature as 230 degrees Fahrenheit and below that the result is not appreciable over the low temperature of mixing.

45 In carrying out my process, I melt the carbonaceous material, such as the fatty substances or organic nitro compounds, or mixtures of the same, as, for example, dinitronaphthalene and trinitrotoluene and add them in fluid condition to the ammonium 50 nitrate, which has been previously heated. I then mix the whole composition thoroughly and during such mixing maintain the temperature above that necessary to maintain the fatty substances or organic nitro 55 compounds in a liquid condition. Prefer-

ably I maintain this temperature as close to the melting point of ammonium nitrate as is safe, and in any event it should be above 230 degrees Fahrenheit. In practice, I have used a temperature of about 280 degrees to 60 290 degrees Fahrenheit with good results. I have, as stated before, obtained better results than in the previous method with a temperature as low as 230 degrees Fahrenheit.

65 An explosive of this character, produced in accordance with my process, will detonate with a much smaller detonator and with more certainty than is the case with such explosives made in the manner that existed 70 prior to my discovery.

75 As an example of my process, I melt 7 parts of dinitronaphthalene with 5 parts of trinitrotoluene and add these in a fluid condition to 88 parts of ammonium nitrate previously heated to a temperature between 280°-290° Fahrenheit. These ingredients are then mixed thoroughly and, during such mixture the temperature is maintained from 280° to 290° Fahrenheit.

80 Having now fully described my invention, what I claim and desire to protect by Letters Patent is—

85 1. The process of producing a high explosive of the character described, which consists in mixing ammonium nitrate with an organic nitro compound at a temperature between two hundred and thirty degrees Fahrenheit and the melting point of the ammonium nitrate.

90 2. The process of producing a high explosive of the character described, which consists in mixing ammonium nitrate with an organic nitro compound at a temperature between two hundred and eighty degrees Fahrenheit and the melting point of the ammonium nitrate.

95 3. The process of producing a high explosive of the character described, which consists in mixing ammonium nitrate with an 100 organic nitro compound at a temperature between two hundred and eighty degrees Fahrenheit and two hundred and ninety degrees Fahrenheit.

105 4. The process of producing a high explosive of the character described, which consists in adding an organic nitro compound, solid at ordinary temperature, in a fluid condition to ammonium nitrate and mixing the same together at a temperature between two 110

hundred and thirty degrees Fahrenheit and the melting point of the ammonium nitrate.

5. The process of producing a high explosive of the character described, which consists in adding an organic nitro compound, solid at ordinary temperature, in a fluid condition to ammonium nitrate and mixing the same together at a temperature between two hundred and eighty degrees Fahrenheit and the melting point of the ammonium nitrate.

10. The process of producing a high explosive of the character described, which consists in adding an organic nitro compound,

solid at ordinary temperature, in a fluid condition to ammonium nitrate and mixing the same together at a temperature between two hundred and eighty degrees Fahrenheit and two hundred and ninety degrees Fahrenheit.

15. In testimony of which invention, I have hereunto set my hand, at Chester, Pa., on 20 this eighth day of August, 1906.

PLUMER WHEELER.

Witnesses:

HAMILTON BRADSHAW,  
HOWARD M. PAULL.